

# UNITED STATES PATENT OFFICE.

HERMAN F. WILLKIE, OF BALTIMORE, MARYLAND, ASSIGNOR TO U. S. INDUSTRIAL  
ALCOHOL CO., A CORPORATION OF WEST VIRGINIA.

## PROCESS OF PRODUCING HOMOGENEOUS PRODUCTS, INCLUDING FILMS.

1,400,196.

Specification of Letters Patent. Patented Dec. 13, 1921.

No Drawing.

Application filed April 12, 1920. Serial No. 373,084.

To all whom it may concern:

Be it known that I, HERMAN F. WILLKIE, a citizen of the United States, residing at Baltimore, in the State of Maryland, have 5 invented a certain new and useful Improvement in Processes of Producing Homogeneous Products, Including Films, of which the following is a specification.

My invention relates particularly to a 10 process of producing homogeneous products of various kinds, but particularly films or coatings from coating compositions containing cellulose esters.

The object of my invention is to provide 15 a process by means of which homogeneous products of various kinds, and particularly films or coatings may be obtained. The object is especially to produce such films or coatings from compositions containing cel-

20 lulose esters, and especially nitrocellulose, which products will be free from cloudiness. Another object is to produce products, and particularly films or coatings in this way from compositions, using as a solvent

25 one or more esters, alcohols, ethers and ketones alone, or mixed together, which are of such a character that the solvent in evaporating will carry off the water contained in the coating composition to such

30 an extent as to obviate leaving behind a product having a cloudy appearance owing to the presence of water. A further object is to use a solvent that will form with water a constant boiling mixture so that the water

35 will most effectively evaporate with the solvent in order to avoid leaving behind a cloudy product of the character above referred to. Still another object is to remove substantially all the water present

40 in the solvent itself in the product dissolved therein, as for example, the cellulose ester, and taken up from the atmosphere owing to the hygroscopic character of the solvent used. Again a further object is

45 to use ethyl acetate as one of the solvent constituents, notwithstanding its great avidity for moisture.

Hitherto, it has not been found possible 50 to produce without the aid of a vacuum films free from cloudiness by the use of merely a low boiling solvent, inasmuch as when the low boiling solvents were previously used, they would evaporate quickly, leaving behind particles of water which 55 would impart to the film a cloudiness. As

a consequence such films were not dense and homogeneous. Furthermore, such films would not take as even color when pigments were present in the coating composition, as the cloudiness which would vary in different 60 portions of the film would produce a variation in the shade of the color used. In order to obviate this effect, it has been customary in the past to include with the low boiling solvent a high boiling solvent, so 65 as to allow the water and low boiling solvent to entirely evaporate before the film became hard. It is one of the objects of my invention to avoid the necessity of using such additional high boiling solvent or solvents. 70

Further objects of my invention will appear from the detailed description thereof contained hereinafter.

While my invention is capable of embodiment in many different forms, for the purpose of illustration I shall describe only 75 certain forms of the same hereinafter.

For example, in carrying out my invention I may make a coating composition by providing a solvent mixture containing— 80

98% by weight of ethyl acetate,  
2% by weight of alcohol, having

a strength of 95%,

in 100 parts by weight of which solvent mixture I may dissolve 8 parts by weight of 85 pyroxylin. In the above composition, the proportions of the ethyl acetate in the solvent mixture may vary considerably, and may be higher or lower, or even as low as 40%, the proportion of the alcohol being increased 90 in that event to 60%. The alcohol may be entirely absent or may be substituted by any other liquid which would not be detrimental to the solvent action of the ethyl acetate, as for example, benzol. It will also 95 be understood that the proportion of the pyroxylin present may be varied to a considerable degree. Instead of the ethyl acetate, I may substitute in part, or as a whole, one or more other substances that may have 100 a dehydrating action, as for example, one or more esters other than ethyl acetate, one or more alcohols other than ethyl alcohol, and one or more ethers or ketones. For example, instead of the ethyl acetate, I may use 105 benzol, amyl acetate, amyl alcohol, iso-butyl alcohol or iso-propyl alcohol. Instead of the pyroxylin, I may use some other cellulose ester, as for example, cellulose acetate or viscose.

The coating composition made in this manner when spread upon a surface to produce a film or coating will rapidly harden until dry, owing to the evaporation of the 5 solvents present. In the evaporation of the ethyl acetate composition, above referred to, the ethyl acetate, alcohol, and water will form a vapor with approximately the composition of the constant boiling mixture containing—

83% by weight of ethyl acetate,  
8% by weight of alcohol,

9% by weight of water,

when there is sufficient alcohol and water 10 present, or

92% by weight of ethyl acetate,

8% by weight of water,

when there is no alcohol present, and the mixture will evaporate, thus removing from 20 the film or coating not only the water present in the solvent mixture, but the water present in the pyroxlin, as well as any water which is taken up by the ethyl acetate during the formation of the film or coating.

25 The film formed in this manner is found to be entirely clear and free from cloudiness. Therefore, films made in this way, and which may have any other desired constituents added thereto, such as pigments, softening

30 materials, body-giving materials, etc., in accordance with the usual practice in the production of films and coatings, will have a uniform color, and will not be lacking in homogeneity due to the presence of bubbles 35 or droplets of water. The solvent which evaporates from the film while the latter is drying or hardening may be recovered in any suitable manner by collecting and condensing the same, and the condensate may

be used over again several times for the production of films. When the solvent mixture has accumulated a considerable percentage of water, however, it may be treated in any suitable manner for the removal of some of the water, so as to permit the solvent 45 mixture to be used over again in the production of films, or the solvent mixture containing water may be used in some other industry without the removal of water therefrom, as for example, extracting oils, 50 fats, and waxes.

Furthermore, it will be understood that my invention is broadly applicable to the production of varnishes, paints or cements as set forth in my application Ser. No. 55 373,083, filed April 12, 1920.

While I have described my invention above in detail, I wish it to be understood that many changes may be made therein without departing from the spirit thereof. 60

I claim:

1. The process which comprises forming a film by evaporating a solution of a cellulose ester in a solvent consisting of an ester having a dehydrating action and an alcohol 65 adapted to form a constant boiling mixture with and carry off water during the evaporation of the solvent.

2. The process which comprises forming a film by evaporating a solution of a cellulose 70 ester in a solvent consisting of ethyl acetate and ethyl alcohol proportioned to form a constant boiling mixture with and carry off water during evaporation of the solvent.

In testimony that I claim the foregoing, I 75 have hereunto set my hand this 11th day of March, 1920.

HERMAN F. WILLKIE.